

# UNITED STATES PATENT OFFICE.

NOAK VICTOR HYBINETTE, OF CHRISTIANIA, NORWAY, AND ROBERT LEE PEEK, OF OTTAWA, CANADA.

## REFINING COPPER-NICKEL MATTE.

1,382,361.

Specification of Letters Patent. Patented June 21, 1921.

No Drawing.

Application filed February 25, 1920. Serial No. 361,275.

*To all whom it may concern:*

Be it known that we, NOAK VICTOR HYBINETTE and ROBERT LEE PEEK, citizens of Norway and the United States, respectively, 5 and residing at, respectively, Christiania, Norway, and Ottawa, Canada, have invented certain new and useful Improvements in Refining Copper-Nickel Matte; and we do hereby declare the following to be a full, 10 clear, and exact description of the invention, such as will enable others skilled in the art to which it appertains to make and use the same.

This invention relates particularly to the 15 separation of copper and nickel by cementation of copper, from a solution containing the two metals, upon a metallic powder containing the same metals, the cementation being carried out without heating the solution 20 above the normal temperature. The process is of particular value in all cyclic processes (such as electrolytic processes) where the same solution is used over and over again, at the normal temperature appropriate 25 to the process, and where a certain amount of acidity has to be maintained in the solution.

It is well known that copper can be cemented upon nickel only under certain 30 conditions, as, for instance, those set forth in United States patents to one of us No. 805,969, and No. 1,128,313, and also, in United States patent granted to Langer and Langer No. 1,291,030. The processes referred to, however, prescribe heating of the 35 solution, and necessitate subsequent cooling if the solution is to be subsequently used at a lower temperature, for example, as an electrolyte, whereas the great expense involved 40 in the heating and subsequent cooling operations is avoided by the present invention, wherein we are able to operate without such heating and subsequent cooling, and without such variations in the strength and 45 concentration of the solution, by evaporation, as result from such heating and cooling operations. Particularly, moreover, as above noted, the process is of value in all cyclic operations, where the same solution 50 is used over and over again, at a normal temperature for such operations, and where a certain concentration and amount of acidity has to be maintained in the solution. Thus, we have found that if, in the cement-

ing out of the copper, the solution is heated 55 to, for instance, 70° C. or above, the acid is, in part at least, neutralized by the metallic nickel employed, and the acidity must then be restored or readjusted in some way, to meet the exigencies of the cyclic 60 operation. So also, if the solution is heated for the cementation, and subsequently cooled, the water lost by evaporation must be replaced or readjusted to maintain proper concentration for the cyclic operation. This 65 readjustment is entirely avoided or reduced to a minimum in our process, because the solution is not heated above the normal temperature, *i. e.*, the temperature at which it is produced or at which it is subsequently 70 to be used, or at which it is to be maintained in the cyclic operation.

In carrying out the process, we grind and roast the bessemerized copper-nickel matte, in much the usual manner, and subject it 75 to treatment with dilute sulfuric acid so as to dissolve out the greater part of the copper present. A certain proportion of the roasted and leached matte is set aside for reduction to metallic powder and is 80 afterward reduced by carbon, hydrogen, carbon monoxid, hydrocarbons, or other reducing agent, preferably at the lowest temperature so that the metallic powder shall be in a correspondingly fine state of subdivision, appropriate to its subsequent use. 85

In the roasting, leaching and reduction operations, it is of advantage to subject the matte to a preliminary coarse grinding for the roasting and leaching and to subject the 90 roasted and leached matte to subsequent finer grinding prior to the reduction. For ordinary purposes, we consider the grinding to 20 mesh or possibly 30 mesh, to be the most advantageous for roasting and leaching, and the subsequent grinding of the roasted and leached powder to about 60 mesh, or possibly even finer, prior to its reduction, in order that the resulting metallic powder may be sufficiently fine to operate to the best advantage in the subsequent 95 cementation operation. But the cementing out of the copper from the solution in which the metallic powder is to be employed will nevertheless proceed to some extent, and a 100 solution free of copper will always be produced even though the roasted and leached matte from which the metallic powder is 105

reduced is not reground after leaching, although in such cases, the operation proceeds with a great deal less economy.

It will be noted that a portion only of the 5 roasted and leached matte is set aside for reduction to metallic powder. The remainder may be dissolved and refined in any one of several ways; for instance, by direct solution in sulfuric acid, or by converting the matte into metal and dissolving the metal, to form a solution or an electrolyte, which may be purified from copper by treatment in the manner described below.

The amount of material set aside or withdrawn 15 for reduction to metallic powder is preferably such that the powder will contain about two parts or more of nickel to every one part of copper contained in the remaining main body portion of the roasted 20 and leached material, which is used to produce the copper-nickel solution to be treated therewith, so that, when the powder is used for the purification of the solution, there will be a large excess of nickel present.

25 To use the metallic powder in cementing out copper from the fairly neutral copper-nickel solution above referred to, it is brought into contact with said solution, at its normal temperature, in such a manner 30 that a large excess of the metallic powder is used in the treatment of an initial portion of the solution and the cementation thus initiated is repeated on fresh portions of the solution until no more copper will cement 35 out without raising the temperature above the normal temperature of the solution. This method of using the metallic powder in the cementation operation is preferably carried out on the counter-current principle. 40 As hereinbefore stated, it is not necessary for a complete precipitation of all the copper to raise the temperature above a normal temperature of the solution (say 40° C. to 60° C.) and, in some cases, it is of great advantage 45 to dispense with the application of heat for other reasons than the cost thereof. In order to produce copper free from nickel, it would be necessary to apply heat, but we do not aim at such purification in the present process. Therefore, for this reason, as well as for other reasons, we stop short of complete exhaustion of the metallic powder, leaving it in a condition wherein it still contains a large amount of metallic nickel 55 which could be used for further cementation if we desired to raise the temperature of the solution.

The metallic copper-nickel material containing the copper cemented thereon, is given 60 an oxidizing roast preferably by mixing it with some of the original copper matte still to be roasted, or even better, by mixing it with partly roasted matte, and then proceeding with the roasting of the mixture. As hereinbefore stated, this me-

tallic material has been ground so fine that it is not well suited for roasting and leaching by itself, since if it were roasted alone, the fine particles of metal would bring about a certain increase in temperature which 70 would cause the metal particles to sinter together and result in incomplete roasting and leaching. By mixing the metallic material with matte, preferably partly roasted, and then proceeding with the roasting of 75 the mixture, this difficulty is obviated and, after the completion of the roasting, the mixture can be leached in the same way as ordinary roasted matte.

The process of the present invention is 80 of more or less general application to the purification of nickel-copper sulfate solutions and electrolytes in order to free them from copper by cementation. It will be noted that an excess of the fine nickel-powder is used and that the cementation operation is carried out at the normal temperature of the solution, so that heating of the solution and subsequent cooling to the normal temperature is avoided. The normal 90 temperature of the solution may be the temperature at which the solution is produced, for example, from a nickel-copper anode, and the purified nickel-sulfate solution, which is freed from copper without material change 95 from the normal temperature, can then be returned to the electrolytic cell and made use of in the further carrying out of the electrolytic process, the entire operation taking place without any material change in temperature from that of the normal temperature of the electrolytic operation. Thus, for example, where the electrolyte is to be maintained at a temperature of about 55° C. during the electrolytic operation, and 100 where an excess of acid is to be supplied with the electrolyte and is present in the impure nickel-copper sulfate solution produced from a nickel-copper anode, the cementation operation can be carried out without any material change in the normal temperature of the solution and the purified solution can be returned to the electrolytic cell without any considerable neutralization 105 of its acidity or material change in its temperature. The process of the present invention is therefore of special value when practised in conjunction with the separation of nickel and copper by electrolysis, as described in the prior U. S. Patent No. 805,969, 110 and in the process of the companion application of one of us Serial No. 358,968. The nickel-sulfate electrolyte, containing an excess of sulfuric acid, may thus be introduced into the cathode compartment of an 115 electrolytic cell and caused to flow through a filtering diaphragm, separating the cathode compartment from the anode compartment, and the impure nickel-copper solution, formed in the anode compartment from a 120 125 130

nickel-copper anode, and containing an excess of sulfuric acid, can then be drawn off and subjected to purification by cementation, in the manner above described, and without material change in its temperature or any considerable change in its acidity, so that the purified nickel-sulfate solution can be returned to the cathode compartment and made use of in the further carrying out of the cyclic process. In its more comprehensive aspect, as above noted, the process of the present invention is of more general application; but the invention is of particular value when combined in a cyclic process in the manner above described. Accordingly, we wish to be understood as claiming the invention in its more comprehensive aspects, as well as in its more specific aspects when combined with a cyclic electrolytic process in the manner above described.

We claim:

1. The method of purifying nickel-copper sulfate solutions from copper by cementation, which comprises bringing the solution into contact with an excess of finely divided nickel at a temperature below that of exhaustion of the nickel; substantially as described.

2. The method of purifying nickel-copper sulfate solutions from copper by cementation, which comprises bringing a nickel-copper sulfate solution containing an excess of free acid into contact with an excess of finely divided nickel at a temperature below that of neutralization of any considerable amount of the acid; substantially as described.

3. The process of separating copper from nickel, which comprises roasting and leaching disintegrated bessemerized nickel-copper matte, reducing the roasted and leached material, and cementing out copper from a nickel-copper solution on an excess of such reduced material, without raising the temperature of the solution substantially above its normal temperature; substantially as described.

4. The method of purifying nickel-copper sulfate electrolytes from copper by cementation, which comprises bringing the electrolyte, while at a temperature appropriate for the subsequent electrolysis thereof, into contact with an excess of finely divided nickel, without raising the temperature of the solution substantially above its normal temperature, and supplying the resulting nickel sulfate solution to the electrolytic process; substantially as described.

5. The method of purifying nickel-copper sulfate electrolytes produced by electrolysis from nickel-copper anodes, which comprises bringing the electrolyte, at substantially the normal temperature of its production, into contact with an excess of finely divided nickel and thereby removing

the copper from the solution by cementation, and returning the purified nickel-sulfate solution without material change in temperature to the electrolytic cell.

6. The method of purifying nickel-copper sulfate electrolytes from copper by cementation and of effecting the electro-deposition of nickel from the purified electrolyte, which comprises supplying the nickel-sulfate electrolyte to the cathode compartment of an electrolytic cell and causing the same to flow through a filter to the anode compartment, dissolving nickel and copper from a nickel-copper anode to form an impure nickel-copper sulfate electrolyte, bringing such electrolyte without material change in temperature, into contact with an excess of finely divided nickel and thereby freeing the solution from copper, and returning the purified electrolyte without material change in temperature to the cathode compartment of the cell.

7. The method of purifying nickel-copper sulfate electrolytes and of separating nickel from the purified nickel-sulfate electrolyte by electro-deposition, which comprises supplying a nickel-sulfate electrolyte containing an excess of free sulfuric acid to the cathode compartment of an electrolytic cell, which cathode compartment is separated from the anode compartment by a filtering diaphragm, causing the electrolyte to flow through said filter to the anode compartment, dissolving nickel and copper from a nickel-copper anode, drawing off the resulting nickel-copper sulfate solution with its excess acid and bringing the same into contact with an excess of finely divided nickel to free the solution from copper by cementation, and returning the purified electrolyte to the cathode compartment of the cell, the cementation operation being carried out without material change in temperature of the solution from the normal temperature of electrolysis; substantially as described.

8. The process of separating copper from nickel, which comprises roasting and leaching disintegrated bessemerized copper matte, reducing the roasted and leached material, and cementing out copper from a nickel-copper solution on such reduced material, using a large excess thereof, and repeating such cementation on fresh portions of nickel-copper solution until no more copper will cement out without raising the temperature of the solution substantially above normal; substantially as described.

9. The process of separating copper from nickel, which comprises roasting and leaching disintegrated bessemerized copper matte, reducing the roasted and leached material, and cementing out copper from a nickel-copper solution on such reduced material, using a large excess thereof, and re-

peating such cementation on fresh portions of nickel-copper solution until no more copper will cement out without raising the temperature of the solution substantially above 5 normal, and then roasting the but partly exhausted metallic material thus obtained; substantially as described.

10. The process of separating copper from nickel, which comprises roasting and leaching 10 disintegrated bessemerized copper matte, reducing the roasted and leached material, and cementing out copper from a nickel-copper solution on such reduced material, using a large excess thereof, and repeating 15 such cementation on fresh portions of nickel-copper solution until no more copper will cement out without raising the temperature of the solution substantially above normal, then mixing the but partly exhausted metal- 20 lic material with further amounts of matte and roasting the mixture; substantially as described.

11. The process of separating copper from nickel, which comprises roasting and leaching 25 disintegrated bessemerized copper matte, regrinding a portion thereof to a fineness greater than is favorable for roasting and leaching, reducing the reground material, and cementing out copper from nickel- 30 copper solution on such reduced material without raising the temperature of the solution substantially above the normal temperature; substantially as described.

12. The process of separating copper from 35 nickel, which comprises roasting and leaching disintegrated bessemerized nickel-copper matte, regrinding a portion of the roasted

and leached material to a fineness greater than is favorable for roasting and leaching, reducing the same, and cementing out copper 40 from a nickel-copper solution on such reduced material, using a large excess thereof, repeating such cementation on fresh portions of nickel-copper solution until no more copper will cement out without raising the temperature of the solution substantially above 45 normal, mixing the but partly exhausted metallic material thus obtained with partly roasted matte and roasting the mixture; substantially as described. 50

13. The method of treating a nickel-copper powder produced by cementation of copper upon nickel without complete exhaustion of the nickel, which comprises admixing 55 such powder with portions of fresh or partly roasted matte, and subjecting the mixture to a roasting operation; substantially as described.

14. The method of separating copper from nickel, which comprises bringing a nickel-copper sulfate solution into contact with an excess of finely divided nickel at a temperature below that of exhaustion of the nickel and thereby producing a product containing a smaller amount of nickel and an increased 60 amount of copper, admixing such product with fresh or partly roasted or rosted matte, and subjecting the mixture to a further roasting operation.

In testimony whereof we affix our signatures. 70

NOAK VICTOR HYBINETTE.  
ROBERT LEE PEEK.